

3,850,978  
SYNTHESIS OF N,N-BIS(2-FLUORO-2,2-DINITRO-ETHYL) CARBAMATES

William H. Gilligan, Washington, D.C., and Mortimer J. Kamlet, Silver Spring, Md., assignors to the United States of America as represented by the Secretary of the Navy  
No Drawing. Filed Nov. 28, 1973, Ser. No. 419,755  
Int. Cl. C07c 125/06

U.S. Cl. 260—482 C

16 Claims

ABSTRACT OF THE DISCLOSURE

Compounds of the formula



are produced by the following reaction sequence:



wherein  $\text{R}_1$ ,  $\text{R}_2$ ,  $\text{R}_3$  and  $\text{R}_4$  vary independently and represent F and  $\text{NO}_2$ ,  $\text{Z}$  represents O and NH, and  $m$  and  $n$  vary independently and are integers from 1 to 2.

BACKGROUND OF THE INVENTION

This invention relates generally to chemical compounds and their production, and more particularly to carbamates and ureas containing nitroalkyl and fluoroalkyl groups.

In the past it has been known to produce N,O-bis(trinitroalkyl) carbamates by condensing a nitro isocyanate with a nitroalkanol. In addition, it has been known to produce N,N'-bis(2,2,2-trinitroethyl) urea by condensing trinitro methane with dimethylolurea. While these "bis" substituted compounds are useful as explosives, they do not possess the explosive energy that "tris" substituted compounds do. Unfortunately, these condensation processes of the prior art are capable of producing only the N,O-bis(trinitro alkyl) carbamates or the N,N'-bis(trinitroethyl) urea, i.e. the processes are not capable of producing either the N,N,O-tris(trinitroalkyl) carbamates or N,N,N'-tris (trinitroethyl) ureas. Moreover, the "N" position of the "bis" carbamates and ureas is so deactivated by the single attached trinitro alkyl group that further substitution is not feasible.

SUMMARY OF THE INVENTION

Accordingly, one object of this invention is to provide new chemical compounds and intermediates for the production thereof.

Another object of this invention is to provide new chemical compounds which are useful as explosives.

A further object of this invention is to provide more powerful explosive compounds.

Yet another object of this invention is to provide powerful explosive compounds having good thermal stability.

A still further object of this invention is to provide a synthesis of high energy explosive compositions.

These and other objects of this invention are accomplished by providing compounds of the formula



wherein  $\text{R}_1$ ,  $\text{R}_2$ ,  $\text{R}_3$  and  $\text{R}_4$  vary independently and can each be F or  $\text{NO}_2$ ,  $\text{Z}$  can be O or NH, and  $m$  and  $n$  are integers which vary independently and can be 1 or 2. These compounds are prepared by a series of reactions culminating in the reaction of compounds of the formula



35 with compounds having either the formula



or



45 under esterifying conditions to produce compounds having the formula



60 or



65 respectively,

70 wherein  $\text{R}_1$ ,  $\text{R}_2$ ,  $\text{R}_3$ ,  $\text{R}_4$ ,  $m$  and  $n$  are as defined above.

## DESCRIPTION OF THE PREFERRED EMBODIMENTS

The synthesis of the compounds of this invention can be outlined by the following scheme:



wherein  $\text{R}_1$ ,  $\text{R}_2$ ,  $\text{R}_3$ , and  $\text{R}_4$  vary independently and are selected from the group consisting of F and  $\text{NO}_2$ ,  $m$  and  $n$  vary independently and are integers of from 1 to 2. The first step in the synthesis is the contacting of a secondary amine of Formula I with carbon tetrachloride in the presence of a  $\text{FeCl}_3$  catalyst to obtain a tertiary amine of Formula II. The tertiary amine of Formula II is then contacted with water, hydrolyzing the trichloro-methyl group, to obtain the corresponding carbamyl chloride of Formula III.

The carbamyl chlorides of Formula III are useful as intermediates in the synthesis of the explosive carbamates and ureas of this invention.

In final step of the synthesis, a carbamyl chloride of Formula III is contacted with a compound of the formula



to obtain an explosive compound of the formula



wherein  $\text{R}_1$ ,  $\text{R}_2$ ,  $\text{R}_3$ , and  $\text{R}_4$  vary independently and are selected from the group consisting of F and  $\text{NO}_2$ , Z is selected from the group consisting of O and NH, and  $m$  and  $n$  vary independently and are integers of from 1 to 2. When Z is O, the final step of the synthesis comprises the contacting of a carbamyl chloride of Formula III with an alcohol of Formula IV to obtain a carbamate of Formula V. On the other hand when Z is NH, the final step of the synthesis comprises the contacting of a carbamyl chloride of Formula III with an amine of Formula VI to produce a urea of Formula VIII. Whether Z is O or NH, this final step involves the reaction of a carbamyl chloride with a compound containing an active hydrogen.

$\text{NO}_2$  groups are necessary for the compounds to be explosives and the fluoro groups provide improved thermal

stability. Therefore, while  $\text{R}_1$ ,  $\text{R}_2$ ,  $\text{R}_3$ , and  $\text{R}_4$  might all be  $\text{NO}_2$ , as in the carbamates



and  
[( $\text{NO}_2$ )<sub>3</sub> $\text{CCH}_2-\text{I}_2\text{NCO}_2\text{CH}_2\text{CH}_2\text{C}(\text{NO}_3)_3$ ],  
or as in the ureas



it is preferable that  $\text{R}_1$  and  $\text{R}_3$  both be F while  $\text{R}_2$  and  $\text{R}_4$  vary independently and are selected from the group consisting of F and  $\text{NO}_2$ . These preferable compounds would, therefore, include carbamates such as



Since the "O" position nitro alkyl or fluoronitro alkyl substitute is added to the carbamate in a separate step, it may be different from the two "N,N" position nitro alkyl or fluoro nitro alkyl substitutes. Thus, mixed carbamates such as



can be prepared. Similarly, since the "N" position nitro alkyl or fluoro alkyl substitute is added to the urea in a separate step, it may be different from the two "N,N" position nitro alkyl or fluoronitro alkyl substitutes. Thus, mix ureas such as



Although the above mixed substituted carbamates and ureas are possible, carbamates and ureas of this invention in which  $m$  and  $n$  both equal 1 are more preferred because they make more powerful explosives than compounds in which  $m$  or  $n$  equals 2. Thus the more preferred carbamates of this invention are



and

$$[(NO_2)_2FCCH_2]_2NCO_2CH_2CF(NO_2)_2$$

with

$$[(NO_2)_2FCCH_2]_2NCO_2CH_2CF(NO_2)_2$$

being the most preferred carbamate. Similarly the most preferred ureas of this invention are



and

$$[(NO_2)_2FCCH_2]_2NCONHCH_2CF(NO_2)_2$$

with

$$[(NO_2)_2FCCH_2]_2NCONHCH_2CF(NO_2)_2$$

being the most preferred urea.

The carbamyl chloride of Formula III may be selected from the group consisting of



Because F substitutes improve the thermal stability of the compounds,



are preferred. More preferred are the fluoro substituted compounds of Formula III in which  $m=1$ , i.e.



being the most preferred carbamyl chloride.

The following examples are given by way of illustration only and are not to be construed as limiting this invention in any manner:

#### EXAMPLE I

##### N,N-bis(2-fluoro-2,2-dinitro ethyl) carbamyl chloride

To a slurry of 16 g. of anhydrous ferric chloride in 105 ml. of carbon tetrachloride, 52 g. of N,N-bis(2-fluoro-2,2-dinitroethyl)amine was added. The mixture was then refluxed for 48 hours with stirring. Next 4 ml. of water in 10 ml. of tetrahydrofuran was added dropwise to the mixture at the reflux temperature over a period of 40 minutes. Refluxing was then continued for an additional hour. The reaction mixture was then taken up in 100 ml. methylene chloride. The methylene chloride solution was then dried over anhydrous magnesium sulfate, filtered, and evaporated in *vacuo*, leaving the product as a residue.

#### EXAMPLE II

##### N,N,O-tris(2-fluoro-2,2-dinitroethyl) carbamate

The residue produced in Example 1 was redissolved in 100 ml. of methylene chloride. To the cooled solution (ice-bath) was added 18 ml. of 2-fluoro-2,2-dinitroethanol. Next, 25 ml. of triethylamine was added to the

cooled solution over a period of 40 minutes. The solution was then allowed to warm up to room temperature and then refluxed overnight. After the solution had cooled to room temperature, the solution was washed first with dilute hydrochloric acid and then with water. Next the solution was dried over anhydrous magnesium sulfate, filtered, and the volatiles were removed *in vacuo*, leaving a residue. The residue was then recrystallized from ether/hexane and finally recrystallized from



to give 42.4 gm. of N,N,O-tris(2-fluoro-2,2-dinitroethyl) carbamate; m.p. 63-5°.

Analysis. Calculated for  $C_7H_6F_3N_7O_{14}$ . C, 17.92; H, 1.29; F, 12.15; N, 20.90. Found, C, 17.88; H, 1.15; F, 12.21; N, 20.78.

Although this invention has been described with reference to but a few preferred embodiments, it should be apparent that it is by no means so limited but, within the scope of the appended claims, it may be practiced in a manner other than as described.

What is claimed as new and desired to be secured by Letters Patent of the United States is:

#### 1. A compound of the formula



wherein  $R_1$ ,  $R_2$ ,  $R_3$  and  $R_4$  vary independently and are selected from the group consisting of F and  $NO_2$ ,  $Z$  is selected from the group consisting of O and NH, and  $m$  and  $n$  vary independently and are integers of from 1 to 2.

2. A compound according to claim 1 wherein  $Z$  is O.

3. A compound according to claim 2 wherein  $R_1$  is F and  $R_3$  is F.

4. A compound according to claim 3 wherein  $m$  equals 1 and  $n$  equals 1.

5. A compound according to claim 4 wherein the compound is



6. A compound according to claim 1 wherein  $Z$  is NH.

7. A compound according to claim 6 wherein  $R_1$  is F and  $R_3$  is F.

8. A compound according to claim 7 wherein  $m$  equals 1 and  $n$  equals 1.

9. A compound according to claim 8 wherein the compound is



#### 10. A compound of the formula



wherein  $R_1$  and  $R_2$  vary independently and are selected from the group consisting of F and  $NO_2$ , and  $m$  is an integer of from 1 to 2.

11. A compound according to claim 10 wherein  $R_1$  is F.

12. A compound according to claim 11 wherein  $m$  equals 1.

13. A compound according to claim 12 wherein the compound is



14. A process for the production of the compounds of claim 1 comprising:

(a) contacting



with carbon tetrachloride to obtain



and contacting



with water to obtain



and (b) contacting



with



to obtain



wherein  $\text{R}_1$ ,  $\text{R}_2$ ,  $\text{R}_3$ , and  $\text{R}_4$  vary independently and are selected from the group consisting of F and  $\text{NO}_2$ ,  $\text{Z}$  is selected from the group consisting of O and NH, and  $m$  and  $n$  vary independently and are integers of from 1 to 2.

15. The process of claim 14 wherein  $\text{Z}$  is O.

16. The process of claim 14 wherein  $\text{Z}$  is NH.

#### References Cited

##### UNITED STATES PATENTS

3,644,519 2/1972 Adolph ----- 260-553 R  
2,978,491 4/1961 Frankel ----- 260-482 C

25 LORRAINE A. WEINBERGER, Primary Examiner  
P. KILLOS, Assistant Examiner

U.S. CL. X.R.

30 149-88; 260-544 C, 553 R, 583